

## UNITED STATES PATENT OFFICE.

ANDREW A. KUCHER, OF CHESTER, PENNSYLVANIA.

## WORKING FLUID FOR REFRIGERATION.

No Drawing. Original application filed April 7, 1922, Serial No. 550,445. Divided and this application filed February 8, 1923, Serial No. 617,844. Renewed April 27, 1927.

This invention relates to the art of refrigeration, particularly as practiced by the so-called compression process, and has for an object to provide an improved working fluid 5 for use in processes of the character designated which shall have as constituents a refrigerant and a lubricant admixing therewith to form a homogeneous fluid of such character that the lubricant is not mechanically segregated from the refrigerant in 10 passing through a compression refrigeration cycle.

Compression refrigerators nominally comprise a chamber in which a working fluid is 15 evaporated at a relatively low pressure and temperature, a chamber in which the vapors are condensed at a higher pressure and temperature, a compression mechanism for translating the vapors from the low-pressure 20 evaporation chamber to the high-pressure condensing chamber, and a valve conduit for returning the condensed fluid at a reduced pressure into the evaporation chamber. The refrigerant fluid thus flows in a 25 continuous cycle during any period of operation, heat being absorbed from the medium surrounding the evaporation chamber in order to secure the desired refrigerating effect, which heat is carried by the refrigerant fluid to the condensing chamber and 30 removed from the apparatus by bringing an outside medium into heat-exchanging relation to the contents of the condensing chamber.

It has been heretofore proposed to employ 35 in compression refrigerators a refrigerant and a lubricant which is immiscible with the refrigerant. Many liquids possessing to a greater or less extent this property have 40 been used, generally with incomplete success, since no combination of refrigerant and lubricant has been found in which the liquids do not mingle to some extent when brought together under the conditions of 45 agitation obtaining in a compression refrigerator. Mechanical separators of various types have been employed with machines of this character to facilitate the separation of the refrigerant and the lubricant. This expedient has improved the operation but has not resulted in accomplishing a sufficiently complete segregation of fluids to enable compression refrigerators utilizing a

compound working fluid of this character to operate for long periods without a replacement of the lubricant.

In the present invention, I provide a compound working fluid for a compression refrigerator which has the properties required of a refrigerant fluid as well as those required for the satisfactory and reliable lubrication of the compression mechanism. In accomplishing this result, I have departed radically from the prior attempts to employ an immiscible refrigerant and lubricant. I have discovered that by the employment of a working fluid comprising a refrigerant and a lubricant which readily mix one with the other to form a physical solution or a homogeneous liquid of a character that its 70 constituents are soluble in each other, I am enabled to overcome completely the lubrication difficulties heretofore experienced in the operation of compression refrigerators.

The refrigerant and lubricant which comprise my admixtures are of such a character that they do not separate out into the segregated bodies under the influence of gravity or of centrifugal action obtaining in a compression refrigerator. In common with admixtures and solutions of this character, a vaporization of one or both of the constituents of my compound working fluid may be effected by temperature or pressure changes thereof. The compound working 85 fluid may thus be considered to consist of a very intimate admixture or a physical solution of its constituent parts.

In obtaining a complete working fluid of 90 this character, a wide range of refrigerants and lubricants may be employed. I have found by experiment that ethyl chloride as a refrigerant and a mineral oil as a lubricant, which oil readily mixes with ethyl chloride, very satisfactorily meet the required conditions for efficient refrigeration and lubrication. Good results have been obtained with a mixture of one part ethyl chloride to one or less parts of mineral oil. The amount of lubricant required depends upon the type of pump employed and upon the character of lubricant utilized. One example of a lubricant which may be satisfactorily employed is a filtered mineral oil 95 having a viscosity of about 700 to 750 seconds at 100 degrees Fahrenheit, Saybolt 100

- universal viscometer, and a pour test of about zero degrees Fahrenheit. An oil of such a character may be mixed with ethyl chloride in an approximate ratio of four parts of ethyl chloride to one part of oil. This admixture has been found under severe centrifugal tests to exhibit no tendencies to separate into its constituents and hence may be said to constitute a true physical solution.
- 10 Another example of a lubricant which may be satisfactorily employed is a filtered mineral oil having a viscosity of about 1500 seconds at 100 degrees Fahrenheit, Saybolt universal viscometer, and a pour test of about 15 degrees Fahrenheit. An oil of such a character may also be mixed with ethyl chloride in an approximate ratio of four parts of ethyl chloride to one part of oil.
- 15 It is to be understood, however, that my invention is not limited to the employment of the particular constituents above mentioned to form the compound working fluid, or to the exact proportions of the constituent refrigerants and lubricants, since it will be obvious to those skilled in the art that my invention is susceptible of various changes and modifications, without departing from the spirit thereof, and I desire, therefore, that only such limitations shall be placed thereupon as are imposed by the prior art or as are specifically set forth in the appended claims.
- 20 What I claim is:
1. A working fluid for a refrigerating apparatus comprising in part ethyl chloride and in part mineral oil forming therewith a true physical solution, the ethyl chloride being equal to or in excess of the mineral oil. 35
  2. As a working fluid for a refrigerating apparatus, a physical solution comprising in part ethyl chloride and in part mineral oil, the ethyl chloride being equal to or preponderating over the mineral oil. 40
  3. A working fluid for a refrigerator comprising ethyl chloride and a lubricant forming therewith a true physical solution. 45
  4. A working fluid for a refrigerator comprising ethyl chloride and a mineral oil forming therewith a true physical solution. 50
  5. A working fluid for a continuous cycle compression refrigerator comprising ethyl chloride and a lubricant forming therewith a true physical solution.
  6. A working fluid for a continuous cycle compression refrigerator comprising ethyl chloride and a mineral oil forming therewith a true physical solution. 55

In testimony whereof, I have hereunto subscribed my name this 30th day of January, 1923.

ANDREW A. KUCHER.